

Q. BENT, E. BARNHART & J. B. LADD.  
METHOD OF TREATING MATERIALS FOR SINTERING.  
APPLICATION FILED JAN. 31, 1913.

1,078,988.

Patented Nov. 18, 1913.



WITNESSES:

*John B. Ladd*  
*Edwin Barnhart*  
*Max Hofmann*

INVENTORS  
Quincy Bent  
Edwin Barnhart  
James B. Ladd  
By *W. G. Co., date*  
their ATTORNEY.

# UNITED STATES PATENT OFFICE.

QUINCY BENT AND EDWIN BARNHART, OF SPARROWS POINT, MARYLAND, AND  
JAMES B. LADD, OF ARDMORE, PENNSYLVANIA.

## METHOD OF TREATING MATERIALS FOR SINTERING.

1,078,988.

Specification of Letters Patent.

Patented Nov. 18, 1913.

Application filed January 31, 1913. Serial No. 745,323.

To all whom it may concern:

Be it known that we, QUINCY BENT and EDWIN BARNHART, citizens of the United States, residing at Sparrows Point, in the county of Baltimore, State of Maryland, and JAMES B. LADD, a citizen of the United States, residing at Ardmore, in the county of Montgomery, State of Pennsylvania, have invented a new and useful Method of Treating Materials for Sintering, of which the following is a specification.

Our invention relates to an improved method of treating materials to be sintered.

The object of the improved method is to 15 prepare the material and deliver the same, in such physical condition as to assure a uniform sintering throughout the entire mass.

Many mineral bearing materials, such as 20 ores, exist in such a finely divided state, like dust or sand, that they cannot be used in metallurgical processes until agglomerated or made into lumps. Such finely divided materials are treated by various processes to 25 reduce them to a useful condition. One process for treatment of such materials is commonly known as sintering. This consists in passing air through the materials, after ignition, thereby causing combustion through the mass to fuse or partly fuse ma- 30 terials therein, and to reduce the mass of fine material to a more or less solid mass suitable for treatment in smelting furnaces or the like. In such cases the combustion is supported either by combustible material 35 originally in the fine ore-bearing material, or by carbon or the like purposely added.

We have found that in sintering these fine materials, which, to be properly agglomerated, must be in a moist state, much better 40 results are secured by separating into small parts the more or less coherent mass of material, and by lightly and evenly sprinkling or depositing said small and separate parts so that the entire mass to be treated shall 45 lie loosely and be of uniform density and consistency. In this condition the mass offers uniform resistance to the passage of air through it, thereby insuring uniform combustion throughout the mass.

50 We have discovered that if the mass is not of uniform consistency, the air will pass more rapidly through the parts which offer the least resistance, and the combustion in

such parts, will be more rapid than in denser parts, and the resulting product will not be 55 uniform, and may not be useful.

We have found that the materials should be not only of uniform consistency throughout, as to resistance to the passage of air, but the particles thereof should also lie 60 loosely. That is to say, the material should not be packed tightly, either as a mass, or in any part of the mass, so as to cause undue resistance to the air current, and thus unnecessarily increase the power required 65 to produce the passage of air through the mass.

Our invention therefore comprises the improved method of preparing the material, or placing the material, in proper physical condition, in position for sintering and like processes. In other words, our method contemplates the final physical treatment of the material preparatory to applying heat thereto.

Referring to the drawings which illustrate merely by way of example, a suitable arrangement for effecting the invention, the figure is a diagrammatic elevation, partly in section.

Referring to this drawing, the pan 1 is provided with the grate 2, which in this case is shown stationary. It is obvious that the grate may be a movable one. Beneath the grate is the suction space or box 3. The 80 sieve or sifter 4 is located above the grate or sintering bed and adapted to deliver material thereto. This sifter is shown as oscillated by the crank 5 and connecting rod 6. It is obvious that a rotating sifter, or any 85 other form of sifter or screen with means for agitating same may be used. Nor need the method herein described and claimed be confined to the use of a sifter or screen. It will obviously include any means suit- 90 able for breaking up the material and sprinkling and depositing the same on a sintering bed in a loose mass of uniform density. Material is delivered to the sifter by the chute 7 delivering from the hopper 8. A 100 feed screw 9 is shown for delivering material from the hopper 8. For the purpose of spreading the material evenly from one end of the pan to the other, the sifter, hopper and chute are shown mounted on a travel- 105 ing crane 10. Of course it will be obvious

that when the grate is a traveling or movable grate, the sifter and associated mechanism may be stationary.

So far as we are aware, in all methods heretofore practised, of sintering these materials, the material is delivered to the pan or grate by a chute, hopper, conveyer or shovel or the like, and no matter how the material has been previously treated, we have found that it cannot be delivered by such methods to form a mass having the desirable characteristics above described by us, namely that the small separated parts lie loosely together, and that the mass has uniform consistency and density throughout.

While ordinarily we consider it preferable to pass the material directly through the screen or sieve to its final resting place in the pan or grate, it will be obvious that any means intervening between the sieve and the pan, which will deliver the material to its final resting place, in such manner as to form a mass having the same desirable characteristics above specified, would come within the spirit and scope of our invention.

It will be understood that we do not use the screen or sieve primarily to size the material, as is usually the object of such devices, but that the primary object of our method is to break up the material and thus reduce it to uniform consistency, and to

deposit it evenly and lightly into a mass of uniform density and consistency to be sintered.

What we claim is:—

1. The method of preparing material for sintering, which consists in sprinkling finely divided moist material and depositing the same directly as sprinkled on a sintering bed in a loose mass of uniform density.

2. The method of preparing material for sintering, which consists in breaking up into small parts finely divided material having a tendency to cohere and depositing the material on a sintering bed in a loose mass of uniform density.

3. The method of preparing material for sintering, which consists in breaking up into small parts finely divided slightly coherent material and depositing the separated parts on a sintering bed in a loose mass of uniform density.

45  
QUINCY BENT.  
EDWIN BARNHART.  
JAMES B. LADD.

Witnesses as to Quincy Bent and Edwin Barnhart:

W. B. HODDINOTT,  
LOUISE B. MORRIS.

Witnesses as to James B. Ladd:

WALTER S. MYERS,  
MAE HOFMANN.